

## UNITED STATES PATENT OFFICE

MAURICE H. ARVESON, OF HAMMOND, INDIANA, ASSIGNOR TO STANDARD OIL COMPANY (INDIANA), OF CHICAGO, ILLINOIS, A CORPORATION OF INDIANA

## MILL GREASE

No Drawing.

Application filed April 28, 1930. Serial No. 448,178.

This invention relates to a lubricant for use on open bearings at high temperatures, such a lubricant being commonly known as mill grease.

5 In cement mills, paper mills, etc. heavy machinery is equipped with open bearings which are lubricated by "bricks" of mill grease. These bearings usually operate at temperatures of 150-250° F., sometimes 10 higher, and the object of this invention is to provide such a mill grease that will withstand more severe operating conditions, higher temperatures and pressures, than greases heretofore known. A further object 15 is to provide a grease of superior wearing qualities. A further object is to provide a process for making such greases which can be easily controlled and which will insure uniformity. A further object is to provide a more efficient process of making grease whereby the cost of manufacture may be reduced. Other objects will be apparent in the following description.

The invention contemplates an improved 25 method wherein the sequence of steps, operating conditions and proportions of materials employed result in a grease of unusually smooth consistency, high melting point, great wearing resistance, and superior quality. A feature of the invention is the complete saponification of tallow or stearic acid prior to the addition of rosin-acid. Another 30 feature is the unexpected abnormal wear resistance offered by a grease having about a one to one tallow-rosin proportion. Another 35 feature is the regulation of the alkalinity by the addition of rosin oil subsequent to the saponification of the tallow. The invention will be better understood from the following detailed description of a preferred embodiment.

In preparing my improved mill grease I may use rosin, rosin oil, or other rosin-acid containing substance; tallow, stearic acid, 45 lard oil, cotton seed oil, oleo stearine, acidless tallow oil, or other fats or fatty acids; viscous hydrocarbon oils of various gravity, flash and viscosity characteristics; and alkalies such as sodium or potassium hydroxide. 50 Rosin-acid is preferably introduced as an

ingredient of rosin oil, which is obtained by digesting rosin in mineral oil at about 500° F. for about 42 hours, using about 30 parts of straw oil (84 second Saybolt at 100° F.) and 70 parts K rosin. The rosin oil prepared in this way contains about 50% rosin-acid.

I may use the ingredients in about the following proportions:

|                                                             |    |
|-------------------------------------------------------------|----|
| 26.2 parts by weight of rosin oil                           | 60 |
| 12.2 parts by weight of tallow                              |    |
| 59.0 parts by weight of oil (500 second Saybolt at 210° F.) |    |
| 3.2 parts by weight of sodium hydroxide                     | 65 |

All of the tallow is mixed with one-half of the oil and all of the sodium hydroxide (which may be dissolved in a small amount of water) in a conventional kettle provided with heating and agitating means. This mixture is heated, with agitation, to a temperature of about 375 to 450° F., preferably about 400° F., until the tallow has been completely saponified.

The rosin oil is next added, the heating 75 and agitation being continued, and the temperature is again raised to about 400° F. (375° to 450° F.) to effect a reaction between the excess alkali and the rosin-acid.

Finally, with continued heating and agitation, the other half of the oil is added and the temperature is again brought to 400° F. (375° to 450° F.). The mixture should be neutral or slightly alkaline at this point and if the reaction is acid, a calculated amount 85 of sodium hydroxide should be added. The grease is then ready to be poured into moulds.

The mill grease prepared by this process is markedly different from and superior to 90 greases formed by the usual process which consists in saponifying a mixture of fatty acid and rosin. Instead of a grainy, soft, low melting composition I obtain a smooth, clear, hard, elastic, high melting mill grease that shows unprecedent wear resistance.

Tests with different rosin-tallow mixtures disclose an unexpected peak in consistency curves. If rosin oil is used, this peak occurs when the amount of rosin oil is a little more than twice the amount of tallow by weight.

- (i. e., when the rosin-acid to tallow ratio is slightly higher than one to one). If rosin is used in this mixture, the peak occurs with a rosin-tallow ratio of one to one. The grease at peak consistency is hard and smooth and it has a high melting point. At peak consistency, the consumption of mill grease reaches a minimum, as shown by numerous experiments and tests at 250 to 260° F.
- 10 The melting point of the grease decreases from 370° F. at 20% rosin to 360° F. at 60% rosin. Greases made with rosin show substantially the same characteristics as those made with rosin oil, the latter however, at peak consistency shows a lower consumption at 250 to 260° F. and a better "top bearing" temperature (the temperature at which the last trace of grease leaves the bearing cup). The "top bearing" temperature for a 50% rosin grease was 330° F. while that of the corresponding rosin oil grease was about 360° F. (within 5° of its melting point).

I believe that an important feature of my invention is the complete saponification of the tallow by the sodium hydroxide prior to the addition of the rosin, the rosin being used to clean up the excess sodium hydroxide and to thereby regulate the alkalinity. I do not limit myself to any theory to account for my phenomenal results, but they are probably due to more complete saponification of fatty acid, less complete saponification of rosin-acid and/or the treatment in at least two distinct steps as hereinabove pointed out.

35 While I have described in detail a preferred embodiment of my invention, it is understood that I do not limit myself to these details except as defined by the following claims.

I claim:

- 40 1. A method of making grease which comprises saponifying a fatty acid with an excess of alkali and subsequently adding a rosin-acid to neutralize the resulting alkalinity.
2. A method of making grease which comprises treating a fatty acid with an excess of alkali at a temperature of from 375 to 450° F., subsequently adding a rosin-acid thereto, and heating the resulting mixture to a temperature of 375 to 450° F.
- 45 3. The process of making a grease which comprises completely saponifying a fatty acid with an excess of alkali and subsequently adding a rosin-acid to utilize the remaining alkali, both steps being carried out in the presence of oil.
- 50 4. The process of making grease which comprises saponifying a fatty acid and subsequently saponifying rosin-acid, the total alkali for the saponification being added to the fatty acid and the saponification thereof being substantially complete before the rosin acid is added to the mixture.
- 55 5. The process of making grease which comprises adding to a fatty acid a quantity of alkali sufficient to saponify said acid and a

substantially equal quantity of rosin-acid, heating the fatty acid and alkali to effect substantially complete saponification, and subsequently adding said rosin-acid and heating the final mixture to saponify said rosin-acid.

6. The process of claim 5 carried out in the presence of oil.

7. The process of making grease which comprises heating a mixture of oil, fatty acid, and excess alkali to a temperature of about 400° F., adding rosin-acid to the hot mixture and again heating to about 400° F., the rosin-acid being proportioned to utilize the free alkali remaining in the mixture.

8. The process of making grease which comprises digesting rosin in oil to form rosin oil, and adding said rosin oil to substantially neutralize an alkaline mixture of saponified fatty-acid in oil.

Signed this 21st day of April, 1930, at Whiting, in the county of Lake, State of Indiana.

MAURICE H. ARVESON.

70

75

80

85

90

95

100

105

110

115

120

125

130